

Nov. 20, 1951

R. J. LEE ET AL.

2,575,718

# METHOD OF PRODUCING POLYOLEFINIC HYDROCARBON DRYING OILS

Filed April 22, 1948



**INVENTORS:**

INVENTORS:  
Robert J. Lee  
Pat S. Drennan

BY Donald E. Payne  
ATTORNEY

## UNITED STATES PATENT OFFICE

2,575,718

METHOD OF PRODUCING POLYOLEFINIC  
HYDROCARBON DRYING OILS

Robert J. Lee, La Marque, and Pat S. Brennan,  
Dickinson, Tex., assignors to Pan American Re-  
fining Corporation, Texas City, Tex., a corpo-  
ration of Delaware

Application April 22, 1948, Serial No. 22,546

3 Claims. (Cl. 260—666)

1

This invention relates to the production of drying oils and other olefinic hydrocarbons by processing high boiling non-aromatic hydrocarbons with HF and it pertains more particularly to novel polyolefin compositions per se and to improved methods and means for obtaining maximum yields of such compositions from charging stocks comprising high boiling paraffins, olefins and/or naphthenes such, for example, as de-aromatized gas oil.

It is known that drying oils can be produced by hydrolyzing hydrocarbon complexes produced in the treating of various hydrocarbons with such compositions as sulfuric acid, aluminum chloride and hydrogen fluoride. Heretofore such processes have lacked commercial feasibility for many reasons; for example, some complexes yield oils of relatively low unsaturation, high specific gravity, undesirable boiling range, and/or other properties which make them unsatisfactory for commercial utilization. An object of this invention is to provide a method and means for producing drying oils of remarkably high unsaturation, containing for example about 4 or more double bonds per molecule, a large portion of which double bonds are in conjugated positions. A further object is to produce polyolefins of lower specific gravity for a given boiling range than that exhibited by prior drying oils produced from hydrocarbon charging stocks. A further object is to provide a new type of synthetic hydrocarbon drying oil which is light in color and which radically differs from any synthetic drying oils of petroleum origin which have heretofore been commercially available. An important object is to avoid or at least to minimize degradation, cracking, polymerization, saturation or other undesirable reactions in the recovery of the drying oil from HF complex material.

A further object of the invention is to provide a process for producing drying oils from a relatively low grade charging stock such as gas oil. A further object is to provide operating conditions for drying oil production which will produce maximum yields of drying oils of desired characteristics while at the same time producing valuable by-product materials. Another object is to provide a relatively simple and inexpensive process for converting hydrocarbons which are higher boiling than gasoline into valuable polyolefinic hydrocarbons, substantially saturated hydrocarbons of the motor fuel boiling range and branched chain saturated hydrocarbons such as isobutane. Other objects will be apparent as the detailed description of the invention proceeds.

In practicing the invention a preferred charging stock is a gas oil which has been de-aromatized by treatment with concentrated sulfuric

2

acid. Many charging stock materials such, for example, as olefin polymers, alkylates, and hydrocarbon fractions produced by carbon monoxide-hydrogen synthesis may contain no appreciable amounts of aromatic hydrocarbons and hence may require no dearomatization step. Relatively pure paraffinic hydrocarbons such as cetane and paraffin waxes may be employed but they give a less desirable product distribution and they are not as commercially attractive as the less valuable gas oils. The dearomatization may of course be effected by other means than treatment with sulfuric acid; the aromatics may be removed by use of known selective solvents but for best results it is important that the aromatic content of the charge be substantially eliminated. The aromatic content should not exceed about 5%, and preferably should be less than about 1%.

The HF treatment of the dearomatized gas oil or other charging stock can be effected at a temperature in the range of about 250 to 450° F., preferably about 300 to 350° F. under a pressure sufficient to maintain liquid phase conditions and with a time of contact which may range from a few minutes to several hours depending upon temperature and intimacy of said contact, excellent results having been obtained with contact times of the order of about 5 to 30, e. g. about 20 minutes. The HF-to-oil ratio may vary from about 0.1:1 to about 5:1 or more but is preferably in the range of about 1:1 to 2:1.

The products of the HF treatment are preferably cooled and separated into an HF phase containing soluble unsaturated hydrocarbons and an insoluble oil phase which consists essentially of saturated hydrocarbons and contains only a small amount of dissolved HF. The oil phase is stripped for removing HF and fractionated to produce motor fuel along with lighter and heavier fractions.

The HF phase separated from the product of the treating step is subjected to a partial stripping operation to remove most of the HF from an HF-polyolefinic hydrocarbon complex without decomposing or degrading said complex. This stripping can usually be effected at temperatures below about 300° F., and in most cases in the range of about 100 to 150° F.; and it may be accomplished by the use of an inert stripping gas and/or by heating. It is important that at least one and preferably one and one-half to two molecules of HF should be left in the stripped residue for each double bond present in the oil components thereof; for practical purposes this means that the stripped residue should contain at least about 30% HF and preferably about 35 to 50% HF by weight. Attempts to recover all of the HF by vacuum distillation or stripping

usually results in serious degradation of the desired unsaturated product.

The stripped complex which contains at least about 1 to 2 molecules of HF per double bond in the hydrocarbon component (i. e. the hydrocarbon product finally produced) is then neutralized with a base, preferably with aqueous ammonia or an aqueous caustic solution. Usually cooling is required in this operation to avoid loss of light ends and to absorb the heat of neutralization. The neutralization may be effected with aqueous ammonia, using adequate cooling so that side reactions are substantially eliminated and neutralization takes place very rapidly without any substantial increase in temperature. 15 The treated complex is thus substantially freed from HF, i. e. it contains less than about 0.1% HF by weight.

The stripped complex may be neutralized by intimate contact with an aqueous caustic solution. Strong caustic solutions may be employed at elevated temperatures (e. g. 100-200° C.) to neutralize the HF, effect isomerization, and give increased yields of a product in which the double bonds are in conjugated position. The neutralized product may then be distilled with inert gas, steam or under vacuum to remove low boiling components therefrom and to produce drying oils either as overhead or as undistilled fractions of desired molecular weight. The drying oils thus produced have remarkably high iodine numbers which usually range from about 450 to 550, from which it may be calculated that they contain 4 to 6 double bonds per molecule (one-third to one-half of which are in conjugated position) and they have remarkably good color. A typical drying oil may have an average molecular weight of about 225, an iodine number of about 475, an ASTM color of about 4, and a maleic anhydride value of about 350. In this connection, iodine number is understood to mean centigrams of iodine per gram of sample as determined by the Wijs' iodine monochloride procedure using 1/2 hour reaction time and 200% excess reagent. Maleic anhydride value represents the milligrams of maleic anhydride which will react with one gram of sample (also referred to as the diene number) and is a measure of the amount of conjugated olefinic double bonds in the samples.

The invention will be more clearly understood from the following detailed description read in conjunction with the accompanying drawings in which:

Figure 1 is a schematic flow diagram illustrating a commercial plant for practicing the invention, and

Figure 2 is a neutralization system utilizable in the system of Figure 1.

Before describing the operation illustrated in the drawings, data will be presented to show the importance and significance of operating conditions. The optimum charging stock appears to be a dearomatized gas oil. The following table sets forth data obtained by treating various charging stocks with a 2:1 HF/oil weight ratio at a temperature of about 330° F. for a contact time of about 20 minutes in an autoclave provided with a motor-driven propellor-type agitator. In these runs, at the end of the reaction period, the reaction mixture was allowed to settle while cooling to room temperature. The lower HF phase was then withdrawn from the bomb through a Saran tube into a neutralizing mixture of aqueous ammonia and cracked ice. The transparent Saran tubing served as a means of

noting when the interface between the acid and the hydrocarbon phases had been reached. The ammonium-fluoride solution was allowed to settle and the poly-olefinic oil was decanted from the solution. The hydrocarbon phase from the reactor was neutralized in a similar fashion and collected separately.

#### Effect of charge stocks

| Charge Stock                | C <sub>18</sub><br>Branched<br>Olefin <sup>1</sup> | C <sub>18</sub><br>Normal<br>Olefin <sup>2</sup> | C <sub>18</sub><br>Branched<br>Paraffin <sup>3</sup> | C <sub>18</sub><br>Normal<br>Paraffin <sup>4</sup> |
|-----------------------------|----------------------------------------------------|--------------------------------------------------|------------------------------------------------------|----------------------------------------------------|
| Vol. Per Cent<br>Conversion | 93-100                                             | (100)                                            | 26.1                                                 | 43.3                                               |
| Yield of Unsat'd<br>Oil     | 38.2                                               | 28.8                                             | 8.9                                                  | 15.2                                               |
| Iodine No.                  | 440                                                | 467                                              | 503                                                  | 475                                                |
| Refractive Index            | 1.526                                              | 1.507                                            | 1.502                                                | 1.498                                              |
| Molecular Weight            | 212                                                | 212                                              | 205                                                  | 213                                                |

| Charge Stock             | C <sub>8</sub><br>Branched<br>2-2-4-Tri-<br>methyl<br>pentane | Dearomatized Gas Oils        |         |
|--------------------------|---------------------------------------------------------------|------------------------------|---------|
|                          | Paraffin <sup>5</sup>                                         | Naph-<br>thenic <sup>6</sup> |         |
| Vol. Per Cent Conversion | 95.7                                                          | 58.7                         | 65      |
| Yield of Unsat'd Oil     | 19.5                                                          | 24.3                         | 22.3    |
| Iodine No.               | 506                                                           | 475                          | 481     |
| Refractive Index         | 1.4910                                                        | 1.517                        | 1.503   |
| Molecular Weight         | 185                                                           | 225                          | 201-229 |

<sup>1</sup> Tetra isobutylene fraction recovered from isobutylene polymer produced by H<sub>2</sub>SO<sub>4</sub> polymerization.

<sup>2</sup> Normal-hexadecene, 95% purity.

<sup>3</sup> Product from complete hydrogenation of (1).

<sup>4</sup> Cetane, 93% purity.

<sup>5</sup> East Texas gas oil (400-650° F. boiling range), dearomatized by exhaustive sulfuric acid treating to a reduced aromatic content of less than 1%.

<sup>6</sup> Hastings gas oil (400-650° F. boiling range), dearomatized by exhaustive sulfuric acid treating to a reduced aromatic content of less than 1%.

When consideration is given to percent conversion, unsaturated oil yield in conversion products, and iodine number of unsaturated oil, it will be noted that the dearomatized gas oils provide a very good charging stock particularly when their cost is compared with that of other charging stocks. The effect of dearomatization is shown by comparative tests on a virgin East Texas gas oil containing about 17% aromatics as compared with the same gas oil after dearomatization by repeated treatment with sulfuric acid. Employing the same treating conditions (2:1 HF-oil weight ratio, 330° F. and 20 minutes contact time) the following comparative data were obtained:

| Charge Stock                                        | Virgin Gas<br>Oil | Dearoma-<br>tized Gas<br>Oil |
|-----------------------------------------------------|-------------------|------------------------------|
| Aromatics                                           | 17.0              | 1                            |
| Volume Per Cent Conversion                          | 40.5              | 59                           |
| Yields (Vol. Per Cent on CH <sub>2</sub> G) Dry Gas | .4                | 1.2                          |
| Isobutane                                           | 4.3               | 12.0                         |
| Normal Butane                                       | .1                | 1.0                          |
| Butenes                                             | .0                | .1                           |
| Pentanes                                            | 2.2               | 6.5                          |
| Pentenes                                            | .4                | 1.0                          |
| C <sub>6</sub> -205° C.                             | 15.1              | 12.9                         |
| Total                                               | 22.5              | 34.7                         |
| Recycle gas oil                                     | 59.5              | 40.7                         |
| HF Soluble Product:                                 |                   |                              |
| Below 205° F.                                       | 1.9               | 4.0                          |
| Gas Oil Range                                       | 5.6               | 11.2                         |
| Heavier than Gas Oil                                | 9.2               | 8.1                          |
| Total                                               | 16.7              | 23.3                         |
| Properties of HF Soluble Oil:                       |                   |                              |
| Iodine Number (Wijs, 1/2 hr.)                       | 297               | 475                          |
| Specific Gravity (65° F.)                           | .9786             | .9059                        |
| Refractive Index (n <sub>D</sub> <sup>25</sup> )    |                   | 1.505                        |
| Gardner Viscosity at 25° C.                         |                   | 1 A-4                        |

The effect of aromatics on the nature and extent of the conversion is strikingly illustrated in the above table. With respect to the HF-soluble

For comparison, properties of the HF-soluble product obtained from the HF treating of de-aromatized gas oil are as follows:

| Cut No.                           | Vol. Per Cent On Chg. | ° C. Ovh.d | Temp. at mm. Hg | Estimated Ovh. Temp. At 760 mm., ° F. | Iodine Number | $n_D^{25}$ | Sp. Gr. At 25° C. | Mol. Wt. |
|-----------------------------------|-----------------------|------------|-----------------|---------------------------------------|---------------|------------|-------------------|----------|
| GASOLINE RANGE MATERIAL           |                       |            |                 |                                       |               |            |                   |          |
| IBP.....                          |                       | 48.5       | 775             | 119                                   |               |            |                   |          |
| 1.....                            | 2.6                   | 100        | 775             | 212                                   | 33            | 1.3860     | .6815             | 102      |
| 2.....                            | 14.6<br>(17.2)        | 110        | 50              | 385                                   | 613           | 1.4665     | .8371             | 132      |
| GAS OIL RANGE MATERIAL            |                       |            |                 |                                       |               |            |                   |          |
| 3.....                            | 16.0                  | 106.5      | 0.9             | 560                                   | 510           | 1.5001     | .9049             | 186      |
| 4.....                            | 16.0                  | 125        | 0.9             | 595                                   | 500           | 1.5081     | .9195             | 220      |
| 5.....                            | 16.0<br>(48.0)        | 154        | 0.8             | 660                                   | 1460          | 1.5165     | .9354             | 256      |
| HEAVIER THAN G. O. RANGE MATERIAL |                       |            |                 |                                       |               |            |                   |          |
| 6.....                            | 11.3                  | 185        | 1.2             | 720                                   | 2445<br>348   | 1.5260     | .9508             | 279      |
| Bottoms.....                      | 23.5<br>(34.8)        |            |                 |                                       |               |            |                   | 379      |
| Total Material.....               |                       |            |                 |                                       | 475           |            | .9059             |          |

<sup>1</sup> Gardner viscosity at 25° C. = A (ca. 50 centistokes or 230 SSU at 25° C.).

<sup>2</sup> Gardner viscosity at 25° C. = L (ca. 300 centistokes or 1460 SSU at 25° C.).

products, the pronounced difference in proportions and particularly in degree of unsaturation is shown by the following comparative data on respective HF-soluble products after neutralization to remove final traces of HF and after removing C<sub>5</sub> and lighter hydrocarbons.

#### HF-soluble products from

| Fraction—Approx. Boiling Range | East Texas Gas Oil |               | Dearomatized Gas Oil |               |
|--------------------------------|--------------------|---------------|----------------------|---------------|
|                                | Per Cent           | Iodine Number | Per Cent             | Iodine Number |
| IBP to 110° C. at 50 mm.       | 12                 | 147           | 17                   | 525           |
| 60°-154° C. at 1 mm.           | 33                 | 315           | 48                   | 485           |
| 154-200° C. at 1 mm.           | 27                 | 255           | 12                   | 445           |
| Bottoms (Tar).....             | 28                 | 181           | 23                   | 348           |
| Total Oil.....                 | 100                | 297           | 100                  | 475           |

A more detailed analysis of the HF-soluble product from the treating of virgin East Texas gas oil is as follows:

| Cut No.                           | Vol. Per Cent On Chg. | ° C. Ovh.d    | Temp. at mm. Hg | Estimated Ovh. Temp. At 760 mm., ° F. | Iodine Number | $n_D^{25}$ | Sp. Gr. At 25° C. | Mol. Wt. |
|-----------------------------------|-----------------------|---------------|-----------------|---------------------------------------|---------------|------------|-------------------|----------|
| GASOLINE RANGE MATERIAL           |                       |               |                 |                                       |               |            |                   |          |
| IBP.....                          |                       | Degrees<br>70 | 765             | Degrees<br>158                        |               |            |                   |          |
| 1.....                            | 1.0                   | 100           | 765             | 212                                   | 48            | 1.4090     | .7258             | 213311   |
| 2.....                            | 10.7<br>(11.7)        | 110           | 46              | 370                                   | 157           | 1.4650     | .8267             |          |
| GAS OIL RANGE MATERIAL            |                       |               |                 |                                       |               |            |                   |          |
| 3.....                            | 16.7                  | 105           | 1               | 555                                   | 336           | 1.5135     | .9086             | 177      |
| 4.....                            | 16.7<br>(33.4)        | 136           | 1               | 620                                   | 293           | 1.5350     | .9384             | 197      |
| HEAVIER THAN G. O. RANGE MATERIAL |                       |               |                 |                                       |               |            |                   |          |
| 5.....                            | 16.7                  | 185           | 1               | 725                                   | 237           | 1.5550     | .9716             | 230      |
| 6.....                            | 10.3                  | 217           | 1               | 800                                   | 273           | 1.5783     | .9976             | 253      |
| Bottoms.....                      | 27.9<br>(54.9)        |               |                 |                                       | 181           |            | 1.0928            | 467      |
| Total Material.....               |                       |               |                 |                                       | 297           |            | .9632             |          |

products obtained from dearomatized gas oil were very surprising.

In addition to the above properties of HF-soluble products produced from dearomatized gas oil it is noteworthy that such products possess a high maleic anhydride value (M. A. V.). For example, cut No. 2 had an M. A. V. of 625 which with its iodine number of 613, mol. weight of 132, and refractive index of 1.4665 indicates a mixture of tri and tetra olefins (3.2 double bonds per mol) which are largely conjugated in structure; i. e. at least 85% of the molecules have one pair of conjugated double bonds. This was qualitatively confirmed by ultra violet spectrophotometric observation. A blend of cuts 4, 5 and 6 showed an M. A. V. of 302, an iodine number of 475, a refractive index of 1.517 and a molecular weight of 250; this indicates that the material is composed of polyolefins containing approximately 4 or more double bonds per molecule and that about 75 to 80% of the material contains one pair of double bonds in conjugation. This is a very unusual combination of properties.

The colors of the vacuum distillate fractions were good varying 1-1½ for the lower boiling components to 3½-5 ASTM for the high boiling products.

For use in the drying oil and/or resin field, cuts 4, 5 and 6 (which represent approximately 43% of the total HF-soluble product) possess the requisite low volatility and adequate body (viscosity) to meet commercial requirements. Each of these fractions air-dry readily and a composite sample produced a slightly less brittle film than a corresponding "polymer" drying oil produced by contacting unrefined cracked gasoline vapors with an absorbent clay under conditions for removing and polymerizing diolefins. Such clay polymer is believed to represent the best drying oils heretofore obtainable from petroleum, but the striking difference between such drying oil and the drying oil of this invention is shown by the following tabulated properties:

|                                                      | Drying oil from HF treating of dearom. gas oil <sup>1</sup> | Drying Oil from Clay Polymer |
|------------------------------------------------------|-------------------------------------------------------------|------------------------------|
| Boiling Range, ° C. at 1 mm. Hg.                     | 106-185                                                     | 104-225                      |
| Refractive Index at 25° C.                           | 1.5178                                                      | 1.5365                       |
| Specific Dispersion (n <sub>F</sub> n <sub>C</sub> ) | 150                                                         | 170                          |
| Specific Gravity at 25° C.                           | 0.9274                                                      | 0.969                        |
| Iodine Number                                        | 439                                                         | 189                          |
| M. A. V.                                             | 302                                                         | 27                           |
| Per Cent Conjugation (from M. A. V.)                 | 77                                                          | 7                            |
| Approximate Mol. Weight                              | 250                                                         | 290                          |
| Viscosity at 100° F.:                                |                                                             |                              |
| Centistokes                                          | 17.28                                                       | 41.7                         |
| Saybolt Universal Sec.                               | 86                                                          | 194                          |
| Color:                                               |                                                             |                              |
| Gardner                                              | 13                                                          | 15                           |
| ASTM                                                 | 4+                                                          | 5                            |
| Drying Time:                                         |                                                             |                              |
| (Set to touch), <sup>2</sup> Hrs.                    | 1½-2½                                                       | 1½-2½                        |
| (Tack-free), Hrs.                                    | 6-8                                                         | 6-8                          |

<sup>1</sup> Composite of cuts 4, 5 and 6.

<sup>2</sup> With 0.5% lead naphthenate and 0.05 cobalt naphthenate driers.

Referring now to the effect of process variables in producing the polyolefin or drying oil materials, the most important are HF/oil ratio, contact time (assuming intimate mixing) and temperature. As the HF/oil weight ratio is increased from about .25:1 to about 3:1 there is a gradual increase in product iodine number and a substantial increase in yield. HF/oil ratios below about 1:1 are usually undesirable not only because of limited yield and lower product unsaturation but because of limited physical capacity of the available HF to dissolve the poly-

olefinic material. The preferred HF/oil ratio is about 1:1 to 2:1 and it is usually uneconomical to employ a greater ratio than 5:1. The properties of the drying oil are not substantially affected by changes in the HF/oil ratio.

The required contact time is dependent on temperature and intimacy of contact; higher temperatures make possible the use of shorter contact times. With an HF/oil ratio of 2 (i. e. 2:1) and a 20 minute contact time, a yield of about 12% is obtained at 265° F. (iodine number 461) while a yield of about 22% is obtained at about 300° F. (iodine number about 510). Adequate conversion at lower temperatures may require a contact time of an hour or more. At higher temperatures, lower HF/oil ratios may be employed advantageously. For example, in a pilot plant run, employing continuous flow type operation at 355° F. and 1:1 HF/oil ratio and 6 to 8 minute contact time, a yield of 12.5 wt. per cent of 474 iodine number oil was obtained. At temperatures of the order of 400° F. the contact time for equivalent conversion may be of the order of about 3-5 minutes. Thus the time of contact may vary from about a minute to an hour or more depending upon the temperature and HF/oil ratio employed but at preferred temperatures such contacting time is in the range of about 5 to 30 minutes. The preferred temperature is in the range of about 300 to 400° F. The iodine number has been observed to decrease with excessively long contact times, said decrease being accompanied by an increase in molecular weight and specific gravity.

Referring now to the drawing, a dearomatized gas oil (or other substantially nonaromatic high boiling hydrocarbon charge) is introduced by line 10 through heater 11 to reactor 12 together with HF introduced through line 13, about 2 parts by weight of HF in this case being introduced per part of oil charge. The reactor may be a batch type or continuous reactor of any known type which will give sufficient intimacy of contact for the required period of time and it is illustrated as a cylindrical vessel provided with a mechanical stirrer 14 driven by motor 15. In the reactor, conversion is effected at a temperature of about 330° F. with a contact time of about 20 minutes under a pressure sufficient to maintain liquid phase conditions, e. g. about 800 to 1500 p. s. i. The charge should of course be dry when it is introduced into the system and conventional drying towers may be employed when necessary. The reactor and other elements must of course be fabricated from or lined with metals, alloys or compositions which are resistant to hydrogen fluoride and may for example be made of Monel or Monel clad. The reactor may consist of a tank provided with a pump-circulated emulsion stream such as employed in conventional sulfuric acid alkylation operations. Since no invention is claimed in the reactor per se it requires no further description.

The reaction mixture is passed through a cooler 16 before being introduced from line 17 to product separator 18. The separator or settler 18 may be operated at substantially reaction pressure but at a temperature below about 250° F. and preferably in the range of about 80 to 180° F. The insoluble saturated oil fraction flows over baffle 19 and is withdrawn through line 20 to stripper 21 which is provided with conventional heating means 22 at its base. Substantially all of the HF dissolved in the hydrocarbon phase is distilled overhead along with light hydrocarbons 75 through line 23 and cooler 24 to HF settler 25

which is preferably operated at a temperature obtainable with ordinary condenser water. Any condensed hydrocarbons separate out as an upper layer and they may flow over baffle 26 and be withdrawn through line 27. A portion of such material may be employed as a stripping gas in stripper 21 and/or in the complex stripper which will be hereinafter described. The net production of the condensed hydrocarbons may be passed through a bauxite tower or otherwise treated to remove HF and/or combined fluorides. Similarly the gas vented from the separator through line 28 may be freed of HF and utilized in any conventional manner. The acid layer is withdrawn through line 29 to HF storage tank 30 from which it is supplied to line 13 by pump 31.

The stripped saturated oil leaves the base of stripper 21 through line 32 and is then fractionated in a conventional system diagrammatically illustrated by tower 33, the light hydrocarbons such as gasoline being taken overhead through line 34 and the heavier hydrocarbons being withdrawn through line 35. Conventional bauxite treating may be used to remove any residual fluorides.

The HF phase from settler 18 which may in this case consist of about 10 to 20 weight percent of unsaturated hydrocarbon material and 80 to 90% by weight hydrogen fluoride is withdrawn through line 36 to HF-complex stripper 37 to which a stripping gas (e. g. from line 27) may be introduced through line 38. Heating means 39 may be employed at the base of this stripper, which operates at temperatures of the order of 125-150° F. The stripping in tower 37 should be sufficient to remove the uncombined HF but to leave at least 1 molecule and preferably 1½ to 2 molecules HF per double bond in the hydrocarbon components contained in the HF solution. In other words, the HF content of the introduced mixture should be reduced to about 35 to 50% by weight but should not be reduced to less than about 30% by weight. Thus a stripped product containing 35 weight percent HF will give an ultimate drying oil of about 450 to 500 iodine number, but if more HF is removed from the material the iodine number of the resulting product gets lower and lower. When stripping is continued to 20% HF content the product iodine number is only slightly above 400. When stripping is continued to 10% HF content, the product iodine number is only about 340. When stripping is continued to .5% HF content, the product iodine number is less than 270. An important feature therefore is to remove the bulk of the HF in this stripping operation without decomposing what is apparently an HF-unsaturated oil complex and to accomplish this purpose, the stripping temperature and pressure should be controlled so that the material leaving the base of the stripper will contain at least 30% and preferably 40 to 50% of HF.

The HF and stripping gas which leaves the top of stripper 37 through line 40 may be combined with the overhead from stripper 21; a part of the overhead may be introduced through branched line 41 into the upper part of stripper 21 and another part may be introduced directly to line 23.

The HF-unsaturated oil complex from the base of stripper 37 may be introduced through cooler 42 and line 43 into a neutralizing system 44 which is shown as a continuous countercurrent tower in Figure 1 and as a multiple batch system in Figure 2. Neutralization is effected by

means of an aqueous neutralizing material or reagent such as ammonia, sodium hydroxide, potassium hydroxide, lime, etc., preferably by aqueous ammonia solution containing from 10 to 20% ammonia. The neutralizing material is introduced through line 45 in sufficient amount to at least neutralize the HF. In the system diagrammatically illustrated in Figure 1, neutralization is effected in a countercurrent tower which may be provided with suitable mixers or contacting surfaces and which may be provided with a series of cooling coils 46, 47 and 48 for temperature control. At the complex inlet end the temperature should be relatively low, e. g. about 30° to 100° F. At the upper end of the tower where the complex has been substantially denuded of combined HF, a higher neutralization temperature of the order of 60 to 150° F. may be employed for removing as much as possible of the combined HF. While the use of a countercurrent system with a temperature gradient as hereinabove described is preferred, it should be understood that the neutralization may be effected at a substantially constant temperature attainable by cooling water, i. e. in the range of 32 to 125° F. or about 85° F.

For obtaining the desired intimacy of contact in the neutralizing step it may be desirable to employ one or more stirred vessels operated batchwise as illustrated in Figure 2. In this case complex from line 43 and aqueous ammonia from line 45 are introduced into stirred mixing vessel 44a which is provided with a jacketed cooler 48a. After intimate mixing for a period of 2 to 20 minutes at about 30 to 125° F. the mixture is introduced by line 49 into batch settler 50. After settling for about 20 minutes the aqueous solution is withdrawn from settler 50 through line 43a and the oil layer is introduced into mixer 44b with additional aqueous ammonia from line 45b. After stirring for another 2 to 20 minutes in this mixer while maintaining a temperature of 50° to 150° F. by cooling jacket 47b the mixture may be introduced by line 49' into settler 50' from which aqueous ammonium fluoride is withdrawn through line 51b and crude drying oil through line 52.

To remove any final traces of HF the crude drying oil may be contacted with bauxite or it may be further neutralized at elevated temperature (e. g. 100-200° C.) with caustic solution introduced through line 53 and intimately mixed with the crude drying oil in mixer 54. The mixture then passes to settler 55 from which the caustic is settled out and withdrawn through line 56, most of the caustic being recycled by pump 57 and a very small amount of spent caustic being withdrawn through line 58. The amount of caustic employed is not critical but it is preferred to employ about .1 to 1 part of concentrated caustic solution since the contacting with caustic in this final neutralization step serves not only to remove the final traces of HF but also to isomerize the olefins and increase the preponderance of conjugated diolefin structure.

The neutralized product may then be distilled under subatmospheric pressure (preferably in the range of 1 to 10 mm.) in conventional distillation equipment illustrated by tower 60, the gasoline boiling range materials being taken overhead through line 61, drying oil distillate being recovered through line 62 and a high boiling polyolefinic drying oil or resin being withdrawn through line 63. Fractions of any desired boiling ranges may thus be obtained. Atmospheric

flash distillation may be employed where the time at elevated temperatures is minimized. A preferred operation is atmospheric distillation in a first tower to remove the lowest boiling component followed by vacuum distillation in a second tower for separation of one or more drying oil fractions.

The drying oil fractions may be utilized directly as such or as a replacement for linseed oil in varnish oils or resins, ink oils, etc., the hydrocarbon nature of the material imparting to any such formulation considerable resistance to water and caustic materials. The fractions also offer utility in core oils, linoleum formulations, binders for pressed wood and fibrous material, plywood laminating agents, paper impregnants, and waterproofing agents. Their conjugated structure enhances their reactivity with other unsaturated compounds. They react with maleic anhydride to form valuable unsaturated dibasic acids or acid anhydrides. The —COOH acid groups thus incorporated in the molecule permit esterification with various monohydric, dihydric and polyhydric alcohols to give a variety of highly useful oils and resins. Certain fractions, particularly the simpler low boiling fractions, offer advantages as raw materials in the chemical industry. Alcohol, acidic groups and the like may be introduced into the molecule by mild oxidation, reaction with halohydrins, nitrogen tetroxide, ketene, sulfonation, etc. The highest boiling fractions may find application in core binders, graphite, electrode binders, asphalt coatings, wood impregnants and the like. A small amount of organically bound fluorine and sulfur may be left in these heavy fractions to impart useful toxic properties. The above are merely illustrative of the many uses to which these new materials may be applied.

From the above description it will be seen that the objects of the invention have been attained. The invention is not limited, however, to the details hereinabove set forth since many modifications of equipment and alternative procedures, conditions and proportions will be apparent from the above description to those skilled in the art.

We claim:

1. The method of obtaining a synthetic drying oil having an average molecular weight of at least about 200, an iodine number in the range of about 400 to 600 and a maleic anhydride value of at least 250, which method comprises contacting a hydrocarbon charging stock which is substantially free from aromatic hydrocarbons with hydrogen fluoride at a temperature in the range of 250° to 450° F. under a pressure sufficient to main-

tain liquid phase conditions with an HF to oil ratio in the range of 1:1 to 5:1 and with a contact time in the range of about 5 to 30 minutes, cooling the contacted materials and separating said materials into a saturated oil phase containing only a small amount of dissolved HF and an HF phase composed chiefly of free HF but containing hydrogen fluoride-hydrocarbon complex in solution, stripping said free HF from the hydrogen fluoride-hydrocarbon complex in the HF phase at a temperature in the range of about 100 to 300° F. and under sufficient pressure to leave at least about one molecule, but not more than 2 molecules, of HF per double bond in the hydrocarbon component of the complex whereby decomposition of said complex is avoided in the stripping step but substantially all uncombined hydrogen fluoride is removed therefrom, neutralizing the HF complex containing at least about 1 but not more than about 2 molecules of HF per double bond in the hydrocarbon component thereof by contacting said complex with an aqueous alkaline solution at a temperature in the range of 30° to 150° F., separating the resulting hydrocarbon and aqueous phases respectively from each other, treating the hydrocarbon phase to eliminate residual amounts of HF and distilling under sub-atmospheric pressure the hydrocarbon phase from which residual HF has been removed.

2. The method of claim 1 wherein the aqueous alkaline solution is an aqueous ammonia solution containing about 10 to 20% ammonia.

3. The method of claim 1 wherein residual HF is removed from the hydrocarbon phase by contacting said phase at a temperature in the range of about 100 to 200° C. with a concentrated caustic solution.

ROBERT J. LEE.  
PAT S. DRENNAN.

#### REFERENCES CITED

The following references are of record in the file of this patent:

#### UNITED STATES PATENTS

| Number    | Name          | Date          |
|-----------|---------------|---------------|
| 2,432,505 | Burk et al.   | Dec. 16, 1947 |
| 2,435,621 | Brooks et al. | Feb. 10, 1948 |
| 2,436,695 | Kuhn          | Feb. 24, 1948 |
| 2,440,459 | Bloch         | Apr. 27, 1948 |
| 2,440,477 | Johnstone     | Apr. 27, 1948 |
| 2,470,894 | Johnstone     | May 24, 1949  |

#### OTHER REFERENCES

Kalichevsky et al., Chemical Refining of Petroleum, pages 49-50 (1942).